

## UNITED STATES PATENT OFFICE

DANIEL STRYKER, OF BROOKLYN, NEW YORK, ASSIGNOR, BY MESNE ASSIGNMENTS,  
TO THE TEXAS COMPANY, OF NEW YORK, N. Y., A CORPORATION OF DELAWARE

## LUBRICATING OIL

No Drawing.

Application filed March 23, 1925. Serial No. 17,797.

This invention has reference to hydrocarbon lubricating oils and relates particularly to compounded lubricating oils, having a hydrocarbon oil as a base, to which has been added a minute amount of an organic material to increase the lubricating properties of the oil.

A substantial proportion of the automobiles now in use are propelled by means of planetary transmission systems in which the cooperating surfaces comprise bands of fabric treated with a proper grade of lubricant. In the course of time the cooperating surfaces of the bands become hard and glazed and fail to operate in the manner originally intended. The result of this is slipping or "chattering" of the transmission bands when starting or stopping, causing uncertainty in the operation of the car in addition to being quite harmful to the bands themselves.

I have found that a great improvement may be derived when operating a car having planetary transmission by employing as a lubricant a hydrocarbon oil containing a minute amount of a natural wax. Such a lubricant is very efficient in preventing chattering of the brake or transmission bands and is easily compounded at low costs.

The natural waxes which have been found to be especially useful in this connection are carnauba wax, bayberry wax, beeswax, japan wax and spermaceti wax. Other natural waxes which are sufficiently soluble in the lubricating oil with which they are to be compounded to prevent actual separation of the wax from the oil may also be employed, but the previously mentioned waxes are specifically pointed out because of their cheapness and availability.

Only minute quantities of these substances are necessary to produce the desired effect. In general, two per cent is the maximum amount necessary to use, while under certain circumstances the amount may be as low as one quarter of one per cent. To prepare the compounded oil it is merely necessary to warm a suitable grade of hydrocarbon oil and stir in the desired amount of the particular wax chosen preferably in a finely divided condition while maintaining the temperature above

normal atmospheric temperature until the wax has entirely dissolved.

While the compounded oils upon which this invention is based are especially well adapted to prevent chattering in planetary transmission automobiles they have also been found to be very valuable for general lubricating purposes. Extensive experiments indicate that compounded oils of this character reduce the wear of metallic parts to a much greater extent than the uncompounded hydrocarbon oil.

In addition oils containing natural waxes are particularly suited for high temperature lubrication such as that obtaining in motor cars owing to the stable character of the waxes, in that they do not break down or become rancid with attendant impairment of the original properties of the compounded oil.

In using the term "natural wax" in the specification and claims I desire it to be understood that I refer to naturally occurring animal and vegetable waxes but do not wish to include naturally occurring mineral waxes, such as ozocerite or other earth waxes which, as far as known, have no special lubricating properties. The waxes specified having been found to have qualities adapted to prevent the chattering in planetary transmissions may be designated as anti-chattering compounds.

What I claim is:

1. A lubricant consisting of a hydrocarbon lubricating oil and a natural wax having anti-chattering properties selected from the following group: carnauba wax, bayberry wax, beeswax, japan wax and spermaceti wax.

2. A lubricant consisting of a hydrocarbon lubricating oil and between 0.25% and 2% of a natural wax having anti-chattering properties selected from the following group: carnauba wax, bayberry wax, beeswax, japan wax and spermaceti wax.

In witness whereof I have hereunto set my hand this 20th day of March, 1925.

DANIEL STRYKER.